

June 2, 1953

L. H. MILLIGAN ET AL

2,640,503

REFRACTORY TUBE

Filed Nov. 21, 1950



*Fig. 1*



*Fig. 2*



*Fig. 3*



*Fig. 4*

Inventors  
LOWELL H. MILLIGAN  
OSGOOD J. WHITTEMORE JR.

By *George L. Lampert*  
Attorney

## UNITED STATES PATENT OFFICE

2,640,503

## REFRACTORY TUBE

Lowell H. Milligan, Worcester, and Osgood J. Whittemore, Jr., Princeton, Mass., assignors to Norton Company, Worcester, Mass., a corporation of Massachusetts

Application November 21, 1950, Serial No. 196,796

4 Claims. (Cl. 138—76)

1

The invention relates to refractory tubes. One object of the invention is to provide a highly refractory tube having high thermal shock resistance. Another object of the invention is to provide a refractory tube having high thermal conductivity. Another object of the invention is to provide a refractory tube having one or more of the above characteristics which is resistant to molten steel.

Another object of the invention is to provide a refractory tube of two concentric portions, in which the two concentric portions have different characteristics adapted for practical use such as beneficiating steel by additions thereto and in which the two portions have similar coefficients of thermal expansion.

Other objects will be in part obvious or in part pointed out hereinafter.

In the accompanying drawings illustrating our invention:

Figure 1 is an axial sectional view of a composite tube in accordance with the invention wherein the silicon carbide portion is on the inside.

Figure 2 is an axial sectional view of a tube according to the invention wherein the silicon carbide portion is on the outside.

Figure 3 is an end elevation of the tube of Figure 1.

Figure 4 is an end elevation of the tube of Figure 2.

For applications where a tube is to be inserted into molten steel for introducing material such as deoxidizers like boron addition agents, or silicon carbide, or purifiers such as calcium carbide thereinto, we provide a composite tube such as shown in Figures 1 and 3 wherein the outer portion 10 is mullite or zircon, and the inner portion 11 is ceramic bonded silicon carbide. Silicon carbide compositions have high thermal shock resistance and high thermal conductivity but will dissolve in molten steel. Mullite and zircon have better resistance toward molten steel but do not have such high thermal shock resistance nor such high thermal conductivity. To obtain the advantages of the several materials the silicate selected from the group consisting of mullite and zircon is placed on the outside where it will contact the molten steel whereas the ceramic bonded silicon carbide is on the inside where it is protected from the molten steel. Thereby deoxidizers or purifiers can be introduced into the steel near the bottom of the melt where they will do the most good. Various additions are made to steel in the ladle. If the ad-

2

ditions are simply dropped into the ladle since cost of them are lighter than steel, they float on top and become part of the slag and have practically no effect so far as beneficiating the steel is concerned. It is desirable to introduce the addition agents near the bottom of the ladle or near the bottom of the molten steel wherever it is to be beneficiated (as perhaps in the open hearth) whereby the beneficiating agent will dissolve in the steel before it has time to rise to the top. Consequently a refractory tube such as shown in Figures 1 and 3 is useful for this purpose for the tube can be pushed well down into the bath of molten steel, in the ladle or otherwise, connected to gas pressure enough to prevent the steel from rising thereinto, and then the addition agent or agents can be run down the tube into the steel, the gas pressure being great enough to cause a slight bubbling and thus to carry the addition agent or agents away from the bottom of the tube.

In other applications for our invention molten steel is allowed to run through the tube. Referring now to Figures 2 and 4, the tube has an outside portion 12 of ceramic bonded silicon carbide and an inside portion 13 of silicate selected from the group consisting of mullite and zircon. Here the silicate resists the attack by the steel, that is to say it will not dissolve therein while the silicon carbide provides desirable thermal shock resistance and thermal conductivity. There are many applications where it is desired to take molten steel from one point to another point by allowing it to flow.

The ceramic bonded silicon carbide may be made in accordance with U. S. Letters Patent No. 2,118,789 of May 24, 1938, to Henry C. Fisher or it can be made as described in U. S. Letters Patent No. 2,515,416 of July 18, 1950, to Lowell H. Milligan. Many other formulae for the ceramic bond are known and may be used. The ultimate bond in many cases includes ceramic bonding constituents derived from impurities in the silicon carbide grain or by reactions with the silicon carbide of the kiln atmosphere during firing. The silicon carbide portion should be at least 50% silicon carbide by weight. We prefer that the portions 11 and 12 be relatively dense, that is having no more than 26% pores by volume.

The material from which the portions 10 and 13 are manufactured is preferably a mixture of particle sizes of zircon or mullite, as the case may be, with ceramic binder. The above particle size mixture which is mostly in the size range coarser than 325 mesh should constitute at least 50% by weight of portions 10 and 13. The ce-

ramic binder may be developed from such materials as clays, bentonite, etc. If bentonite is used as little as 1% or 2% may give a strong product, but useful articles can be made having as much as 20% ceramic material such as clay or a mixture of clays with or without the addition of one or more fluxes or fillers. We may use a small amount of temporary binder, such as dextrine, to give the articles "green" strength, and of course this burns out during the firing.

The manufacturing procedure may be to fill a rubber lined hydraulic mold having a steel core rod with one mixture, apply the hydraulic pressure to compress this mixture, release the hydraulic pressure which will cause the rubber liner to expand again, fill the remaining space with the second mixture, apply the pressure a second time, remove the pressed composite tube from the mold, dry it, then fire it at cone 16. Hydraulic molding with flexible rubber liners is now well known so it need not further be described herein.

The silicon carbide is of course a product of the electric furnace and any commercial grade of silicon carbide can be used. Commercial grades vary from 95% to better than 99% pure. Naturally the purer varieties are preferable but are also a little more expensive and the less pure grades will give satisfactory results in this invention.

Mullite is a compound of the formula  $3\text{Al}_2\text{O}_3 \cdot 2\text{SiO}_2$ . Although it rarely occurs in nature it can be synthesized in the electric furnace. In practical mullite materials there may be excess alumina which may exist as alpha alumina or excess silica which may exist as siliceous glass. Mullite may also be developed by calcining alumino silicate minerals in which case X-rays may show that more mullite exists than is indicated by microscopic examinations.

Zircon is zirconium silicate  $\text{ZrSiO}_4$ . It is found in nature and can be fused and purified in the electric furnace.

One desirable characteristic of our composite tube is that each of mullite and zircon have coefficients of thermal expansion close to that of ceramic bonded silicon carbide. Consequently tubes made in accordance with this invention will not crack during use as indicated above nor will the outer portion separate deleteriously from the inner portion when the composite tube is heated and cooled.

It will thus be seen that there has been provided by this invention a refractory tube in which the various objects hereinabove set forth together with many thoroughly practical advantages are successfully achieved. As many possible embodiments may be made of the above invention and as many changes might be made in the embodiment above set forth, it is to be understood that all matter hereinbefore described or shown in the accompanying drawings is to be interpreted as illustrative and not in a limiting sense.

We claim:

1. A refractory tube consisting of at least two portions concentrically related and integrally joined, one of said portions being inner of the other of said portions, one of said portions being of ceramic bonded silicon carbide, said ceramic bonded silicon carbide portion being at least 50% by weight silicon carbide, said other portion being at least 50% by weight silicate, said silicate being selected from the group consisting of mullite and zircon.

2. A refractory tube consisting of at least two portions concentrically related and integrally joined, one of said portions being inner of the other of said portions, one of said portions being of ceramic bonded silicon carbide, said ceramic bonded silicon carbide portion being at least 50% by weight silicon carbide and having not more than 26% pores, said other portion being at least 50%, by weight silicate, said silicate being selected from the group consisting of mullite and zircon.

3. A refractory tube according to claim 1 in which the silicon carbide portion is inside of the silicate portion.

4. A refractory tube according to claim 1 in which the silicon carbide portion is outside of the silicate portion.

LOWELL H. MILLIGAN.  
OSGOOD J. WHITTEMORE, JR.

References Cited in the file of this patent

UNITED STATES PATENTS

| Number    | Name         | Date          |
|-----------|--------------|---------------|
| 1,949,731 | Soldatoff    | Mar. 6, 1934  |
| 2,308,307 | Robinson     | Jan. 12, 1943 |
| 2,408,467 | Lyons        | Oct. 1, 1946  |
| 2,447,672 | Smith et al. | Aug. 24, 1948 |